

United States Patent [19]  
Gabrusenok

[11] 3,844,832  
[45] Oct. 29, 1974

[54] **METHOD OF MANUFACTURING A HYDROSENSITIVE ELEMENT FOR A HUMIDITY SENSITIVE DEVICE**

|           |        |              |          |
|-----------|--------|--------------|----------|
| 2,876,321 | 3/1959 | Amdur .....  | 236/44 E |
| 2,937,524 | 5/1960 | Gregor ..... | 324/65 R |
| 3,175,400 | 3/1965 | Amdur .....  | 236/44 E |

[76] Inventor: Pavel Stepanovich Gabrusenok,  
Sadovaya ul. 24, kv. 12, Leningrad,  
U.S.S.R.

[22] Filed: May 14, 1973

[21] Appl. No.: 360,167

**Related U.S. Application Data**

[60] Continuation-in-part of Ser. No. 160,699, July 8, 1971, abandoned, which is a division of Ser. No. 776,969, Nov. 19, 1968, Pat. No. 3,712,860.

[52] U.S. Cl..... 117/219, 117/115, 117/164, 117/933, 73/335, 73/338, 236/44 E, 324/65 R

[51] Int. Cl..... B44d 1/18

[58] **Field of Search** ..... 117/215, 217, 219, 164, 117/115, 201, 113, 933; 324/65 R; 73/335, 338; 236/44 E

[56] **References Cited**

UNITED STATES PATENTS

2,377,426 6/1945 Kersten..... 324/65 R

*Primary Examiner*—Ralph S. Kendall  
*Assistant Examiner*—Michael F. Esposito  
*Attorney, Agent, or Firm*—Waters, Roditi, Schwartz & Nissen

[57]

**ABSTRACT**

A hygrosensitive element is produced by passing a flexible, smooth, dielectric film uniformly and continuously in succession through a solution of gelatin and then through an aqueous solution of a hygroscopic salt and a tanning agent for the gelatin. A layer of gelatin of uniform thickness is formed on the film and the salt is uniformly distributed throughout the gelatin layer. The layer is dried, exposed to light to tan or harden the gelatin and then the strip is cut into separate film elements.

9 Claims, 2 Drawing Figures



PATENTED OCT 29 1974

3,844,832

FIG. 1



FIG. 2



**METHOD OF MANUFACTURING A  
HYDROSENSITIVE ELEMENT FOR A HUMIDITY  
SENSITIVE DEVICE**

**CROSS-REFERENCE TO RELATED  
APPLICATIONS**

This application is a continuation-in-part of application Ser. No. 160,699, filed July 8, 1971, now abandoned, which in turn is a divisional of application, Ser. No. 776,969, filed Nov. 19, 1968, now U.S. Pat. No. 3,712,860.

**DETAILED DESCRIPTION**

The present invention relates to a method for manufacturing a hygroscopic element for electrolytic humidity responsive devices used in combination with appropriate electrical circuitry in systems for remote measurement, recording and automatic control of humidity in air-conditioning systems and other installations.

Such humidity sensitive devices will be referred to as "air-humidity detectors" and it is to be understood that they are applicable to the measurement of the humidity of other gases too, provided they do not attack the materials of the detector.

The electrolytic air humidity detectors known in the art comprise a base or backing or support with electrodes rigidly fastened thereto and a hygroscopic coating applied to the base over the electrodes, said coating containing a hygroscopic salt and a film-forming binding agent. In such a case the hygroscopic element is an integral part of the detector. This, as will be explained below, is the main cause of insufficient stability and interchangeability of the currently used electrolytic air-humidity detectors.

One of the main objects involved in increasing the stability and interchangeability of the electrolytic detectors amounts to making a hygroscopic coating of uniform thickness and concentration and retaining this uniformity in the course of operation. This object cannot be achieved unless the process of application of the hygroscopic coating is continuous for each batch of detectors because the beginning and end of each process are inevitably marked by some transitional steps exerting a different effect in each particular case on the thickness of the coating applied.

Besides, the hygroscopic coating must be applied to a homogeneously smooth surface which is free from cracks, sharp changes of shape, joints between different materials, otherwise the capillary forces and adhesion gradient on the base surface may lead to local thickening of the applied coating and to displacement of the hygroscopic substance during detector operation owing to inconstancy in time of the capillary and adhesion forces.

Of the known methods of application of the hygroscopic coating the most commonly used are methods in which each detector is dipped into a film-forming hygroscopic solution and uniformly withdrawn therefrom, or the solution is applied to the surface of the detector with a brush.

The above methods fail to ensure high-quality hygroscopic coatings of the air-humidity detectors.

Intermittent application of the coating, irregular surface, and heterogeneous materials on the surface of detectors (electric insulating base and metal electrodes) preclude the production of a hygroscopic coating of

uniform thickness and fail to ensure the constancy of thickness in the course of detector operation which necessitates individual calibration and setting of each detector during manufacture and leads to insufficient stability of calibration characteristics in time.

It is, therefore, an object of the present invention to provide a method for producing a hygroscopic element featuring high stability and interchangeability.

Another object of the present invention is to provide a method of batch production of said hygroscopic elements.

Still another object of the invention resides in providing an electrolytic detector capable of using the above described hygroscopic elements.

15 With these and other objects in view, the present invention aims at providing a method for producing a hygroscopic element with a homogeneous smooth surface of the base and a hygroscopic coating of uniform thickness, said element being a separate detachable 20 part of the detector, said method ensuring continuity of application of the hygroscopic coating to the element base.

This objective is achieved by providing a method in which a hygroscopic element has its coating uniformly applied to a homogeneous, flexible dielectric film.

The flexibility of the backing makes it possible to apply uninterruptedly the hygroscopic coating to a continuously moving strip, while the homogeneity of 30 said strip ensures stability of the coating thickness along the strip length.

It is practicable to provide for rigid connection of and electric contact with the hygroscopic element by the use of electrodes placed on the hygroscopic element.

35 A method of manufacturing hygroscopic elements according to the invention consists in pulling a flexible strip, e.g., a dielectric film, continuously and at a uniform speed through a solution of gelatin to form a gelatin layer of uniform thickness on said film which layer 40 is then impregnated with an aqueous solution of hygroscopic salt and an added tanning component so that the salt is spread uniformly throughout the layer of gelatin. Then the obtained coating is dried, exposed to light for tanning of the gelatin and cut into separate film elements.

45 A broad range of well known hygroscopic substances can be used as the hygroscopic salt. In particular, suitable substances are lithium chloride  $\text{LiCl}$ , zinc chloride  $\text{ZnCl}_2$ , calcium chloride  $\text{CaCl}_2$ , magnesium chloride  $\text{MgCl}_2$ , and a mixture of potassium-sodium tartrate with sodium chloride  $\text{KNaC}_4\text{H}_4\text{O}_6 \cdot 4\text{H}_2\text{O} + \text{NaCl}$ .

50 Suitable tanning components that can be used are potassium bichromate, ammonium bichromate, formalin, chromium acetate  $\text{Cr}(\text{CH}_3\text{COO})_3$ , the diglycidic ester of ethylene glycol  $\text{CH}_2\text{CHO} \cdot \text{CH}_2\text{OCH}_2 \cdot \text{OCH}_2 \cdot \text{CHOCH}_2$ , and mucochloric (dichloroformylacrylic) acid  $\text{Cl} \cdot \text{C}(\text{COH}) \cdot \text{CCl} \cdot \text{COOH}$ .

55 For applying the hygroscopic coating it is preferred to pull the film through a 10 percent solution of gelatin at a temperature of  $36^\circ\text{C}$ . then through the aqueous solution of hygroscopic salt and tanning component. The temperature of the gelatin solution is maintained at  $36^\circ\text{C}$ . because the solution has the maximum viscosity at this temperature, and, consequently, the temperature dependence of the viscosity is minimum.

60 Now the invention will be better understood from a description of an embodiment given by way of example

of a hygrosensitive element and detector with reference to the accompanying drawings in which:

FIG. 1 shows a hygrosensitive element of the present invention; and

FIG. 2 is a sectional view of an air-humidity detector with the element of FIG. 1.

A hygrosensitive element 1 has a film support (FIG. 1) comprising a triacetate, nitrocellulose, or other flexible strip whose surface is covered with a hygrosensitive coating 15 to 20 microns thick.

Glued to the ends of the hygrosensitive elements are two electrodes 2 made from anti-corrosion metal foil.

The electrolytic air-humidity detector comprises an electric insulating base 3 (FIG. 2) to which a hygrosensitive element 6 is fastened by contact plates 4 and screws 5. On top, the detector is provided with a protective casing 7 with a fine-meshed metal screen 8.

The hygrosensitive elements are manufactured, according to the invention, as follows:

A triacetate, nitrocellulose, or other support of photographic film (provided with a prime or bonding layer) in the form of a long strip moving around a cylindrical shaft and contacting at one side a 10 percent aqueous solution of gelatin at 36°C. is pulled through said solution at a uniform speed of 300 cm/min so that the surface of the backing becomes covered with a layer of gelatin 15 to 20 microns thick, accurate within 5 percent. Then, after the coating is dried, the film is then pulled through an aqueous solution of lithium chloride with a specific gravity of from 1.032 to 1.065 g/cm<sup>3</sup> at 20°C. with the addition of 5 to 20 ml of aqueous solution of potassium bichromate saturated at 20°C. per litre of said first named solution. The strip is pulled at a speed of 1 cm/min, the solution temperature being 10° to 18°C. so that the gelatin is impregnated with the solution to three-fourths of its thickness. Then the gelatin coating is dried in the course of 5 minutes at 50° to 80°C. being simultaneously exposed for 30 minutes to the light of a conventional 100 W incandescent lamp placed at a distance of 50 cm from the film.

The dried film is cut into strips of equal lengths and width and the ends of these strips are provided with glued-on plates 0.05 to 0.1 mm thick made of gold or silver foil.

By pulling the film in succession through the film-forming and hygroscopic solutions, it is possible to ensure a high uniformity of distribution of lithium chloride over the area of gelatin coating while in the previous one stage coating, the film which is pulled only once through a mixture of the film-forming and hygroscopic solutions prevents the gelatin from being used as a film-forming agent; gelatin in this case loses its gelling ability which affects adversely the uniformity of coating thickness.

In lieu of the lithium chloride, other suitable hygroscopic substances can be employed, and in similar respects other suitable tanning agents are equally applicable.

Moreover, it is equally possible to employ polyvinylacetate instead of gelatin.

Also, the influence of a light is obligatory for hardening gelatin, however, it does not necessarily represent an independent step of the process. Namely, if all the operations are carried out in the light, this usually is

sufficient. Moreover, the term "light" is intended to cover UV light as well.

The speed of pulling the film through the gelatin solution could be substantially reduced still maintaining the same concentration of gelatin in the solution. In this case the gelatin layer formed on the film will be substantially thinner. When pulling at a speed of 5 cm/min the gelatin layer will be about 1 micron thick. This embodiment of the method results in somewhat reduced stability of the produced hygrosensitive elements, but at the same time substantially improves the quick-response characteristic thereof (due to reduced inertia).

Inasmuch as the above described hygrosensitive element and detector and the method of their manufacture may vary within the spirit and scope of the appended claims it will be understood that the description above does not restrict the invention to these particular embodiments which have been disclosed.

What is claimed is:

20. 1. A method of manufacturing a hygrosensitive element comprising pulling a flexible strip in the form of a dielectric film continuously at a uniform speed through a solution of gelatin for producing on the film a uniform gelatin layer, impregnating the gelatin layer with an aqueous solution consisting of a hygroscopic salt and a tanning component such that the salt is distributed uniformly in the gelatin layer, drying the coating, exposing the coating to light for tanning the gelatin and cutting the strip into separate film elements.
25. 2. A method according to claim 1 wherein the solution of gelatin is a 10 percent aqueous solution, said solution being kept through at a constant temperature of 36°C.
30. 3. A method according to claim 2 wherein said strip is successively pulled through said solution of gelatin and the aqueous solution of hygroscopic salt and tanning component.
35. 4. A method according to claim 2 wherein said strip is pulled through said gelatin solution at a speed to form a gelatin layer 15 to 20 microns thick, said strip coated with gelatin then being pulled through the aqueous solution of hygroscopic salt and tanning component so that the gelatin is impregnated to three-fourths of its thickness.
40. 5. A method according to claim 4 wherein the strip speed through the gelatin solution is 300 cm/min and through the aqueous solution of hygroscopic salt and tanning component is 1 cm/min, the temperature of the latter solution being 10° to 18°C.
45. 6. A method according to claim 1 comprising drying said gelatin layer on said film before drawing the film through the solution of hygroscopic salt and tanning component.
50. 7. A method according to claim 1 wherein said hygroscopic salt is lithium chloride, zinc chloride, calcium chloride, magnesium chloride, or a mixture of potassium sodium tartrate with sodium chloride.
55. 8. A method according to claim 1 wherein said tanning component is potassium bichromate, ammonium bichromate, formaline, chromium acetate, the diglycidic ester of ethylene glycol or mucochloric acid.
60. 9. A method according to claim 1 wherein said aqueous solution of hygroscopic salt and tanning agent consists of a solution of lithium chloride with a specific gravity from 1.032 to 1.065 g/cm<sup>3</sup> at 20°C. and 5 to 20 ml, per liter of solution, of an aqueous solution of potassium bichromate saturated at 20°C.

\* \* \* \* \*

UNITED STATES PATENT AND TRADEMARK OFFICE  
CERTIFICATE OF CORRECTION

PATENT NO. : 3,844,832  
DATED : October 29, 1974

INVENTOR(S) : Pavel S. Gabrusenok

It is certified that error appears in the above-identified patent and that said Letters Patent are hereby corrected as shown below:

**In the Title:**

Change "hydrosensitive" to --hygrosensitive--

Column 4, line 14, change "hydrosensitive" to --hygrosensitive--

Claim 1, line 1, change "hydrosensitive" to --hygrosensitive--

Column 1, line 64, change "dectectors" to --detectors--

Column 3, line 10, change "mincrons" to --microns--

Claim 2, line 3, cancel "through"

**Signed and Sealed this**

*Sixth Day of December 1977*

[SEAL]

*Attest:*

**RUTH C. MASON**

*Attesting Officer*

**LUTRELLE F. PARKER**

*Acting Commissioner of Patents and Trademarks*